

Patented Sept. 13, 1927.

1,642,309

# UNITED STATES PATENT OFFICE.

WILLY PIEPER, OF NUERMBERG, GERMANY, ASSIGNOR TO J. B. SOELLNER NACHF.  
REISSLZEUGFABRIK A.-G., OF NUERMBERG, GERMANY.

## PROCESS FOR THE PRODUCTION OF A WEATHERPROOF OXIDE LAYER ON ELECTRON METAL.

No Drawing. Application filed May 22, 1924, Serial No. 715,251, and in Germany July 4, 1923.

The surface of the commonly used electron metal i. e. of a manganese base zinc-aluminum alloy which as regards quality, weight and appearance is similar to aluminum, is not weather-proof but changes under the action of the atmospheric air after a short time. Numerous processes have been invented with the view to do away with this disagreeable property of this metal by producing a weather-proof protecting coating on the metal by oxidation. The known processes give however no satisfactory result as they all use acid solutions.

According to this invention no acid solution but an alkaline solution is used in combination with substances which give off oxygen, whereby a thick coating of oxide is produced. The precise dimensions of the finished article are not at all altered by this oxide layer. The oxide layer is absolutely weather-proof, adapted to be burnished and to permit, for the first time, the coloring of electron metal, this coloring adhering not only on the surface of the oxide coating but permeating through the entire layer of oxide.

The process according to this invention may for instance be carried through in the following manner:

The electron metal or the articles made from it are dipped into an alkaline solution heated to approximately 110 to 120° C., for instance sodium hydroxide, in combination with substances which give off oxygen, for instance potassium nitrate, ferric hydrate or the like. When the articles to be oxidized are being dipped into the alkaline solution they are preferably slightly moved to and fro.

After a short time a very uniform oxide coating is produced which strongly adheres to the fundamental metal and is of grey color, that is of similar appearance as the electron metal. After an immersion of about 20 minutes the oxide coating is for instance 0,05 mm. thick; it may however be produced at a thickness of 0,30 mm. and more. The electron metal is dried after it has been taken out of the solution whereupon the oxide coating may be burnished.

The oxide coating may be colored by alkaline proof coloring substances of any kind, preferably by means of aniline dyes. The dyes are preferably added to the alkaline

solution so that the oxide coating produced is colored. The oxide coating may however be colored later on after the drying of the electron metal by separate treatment with alkaline proof solution of dyes and metal oxides.

The coloring substance permeates the entire oxide coating so that the coloring is quite as durable as the oxide coating.

By the above described treatment of the electron metal with a hot alkaline solution in combination with substances giving off oxygen the structure of those parts of the metal is changed which is permeated by the solution and the coloring substance can permeate this changed layer of the metal.

To produce multi-colored oxide coatings, coloring substances soluble in oil, which preferably are also alkaline proof, and to which oil, wax, vaseline, paraffin, or any other fat of viscous consistency is added, are painted in the desired design on the metal article having the oxide coating, whereupon the metal article with the paint is heated for about 10 seconds at a temperature of about 150° C. and cooled slowly. The coloring substance will then have permeated the entire oxide layer so that it is as lasting as this layer. The metal thus treated may be burnished.

The color is preferably put on with the aid of a stencil so that designs of any kind and colors can be produced with sharp outlines or not. Very effective multicolor effects can thus be produced.

The finished colored or uncolored oxide layer may be subsequently impregnated with hydrocarbons, oils or the like to make the same to a higher degree resistant against the influences of the weather or even waterproof. As the structure of the metal has been altered at the production of the oxide layer the hydrocarbons, oils or the like can penetrate into the metal, like the coloring substances.

The above described process may further be used for other metals possessing similar properties as the electron metal. This process is however especially important for the manufacturing of slide rules of metal, as they can be colored in the same manner as the wood slide rules. The parts of a metal slide rule corresponding to the parts at

which the wood is visible in wooden slide rules are colored brown and the parts of the metal slide which correspond to the parts of the wooden slides covered with celluloid are 5 colored grey so that the metal slide rule looks exactly like a wooden slide rule.

I claim:—

1. A process of producing a weather-proof protecting coating on electron-metal 10 and similar metals by oxidation, consisting in using for the oxidation a solution of sodium hydroxide and of chemical substances giving off oxygen, such solution containing

potassium nitrate, said solution being free from any oily matter. 15

2. A process of producing a weather-proof protecting coating on electron-metal and similar metals by oxidation, consisting in using for the oxidation a solution of sodium hydroxide and of chemical substances giving off oxygen, such solution including ferric 20 hydrate, said solution being free from any oily matter.

In testimony whereof I affix my signature.

WILLY PIEPER.